

## UNITED STATES PATENT OFFICE

HARRY C. CLAFLIN, OF CLEVELAND, OHIO, ASSIGNOR TO BERYLLIUM DEVELOPMENT CORPORATION, OF NEW YORK, N. Y., A CORPORATION OF DELAWARE

## PROCESS FOR PRODUCING BERYLLIUM METAL

No Drawing.

Application filed January 3, 1931. Serial No. 506,498.

This invention relates to the manufacture of beryllium metal and its primary object is to make such manufacture both simple and economical.

5 The nature, objects and advantages of the invention will be best understood from the following brief description of earlier methods.

The methods heretofore employed in the 10 isolation of elementary beryllium have involved the electrolysis of a beryllium halide in the presence of one or more halides of metals more electropositive than beryllium, notably sodium or barium. Of the methods 15 already known, the electrolysis of beryllium chloride in the presence of another chloride is probably the most economical. Such a procedure requires, for the electrolysis itself, no apparatus uncommon to general pyro- 20 electrometallurgy, and its electrolysis chemical and energy costs are also low enough to be commercial.

One of the primary objections to this 25 general method of manufacturing beryllium, however, is the difficulty of preparing the anhydrous beryllium chloride necessary for the electrolysis. Dehydration of the hydrated chloride in the presence of ammonium chloride and sodium chloride, as first suggested by

30 Borchers, yields only a semi-fusible mass almost entirely hydrolyzed to beryllium oxide, the chlorine being lost by hydrolysis in the form of HCl gas. Such a mass cannot yield pure metal, if it can give any metal at all, 35 which is highly questionable. It is, therefore, necessary to prepare beryllium chloride by strictly anhydrous processes. From beryllium oxide or carbonate, the compounds of beryllium most common the convenient, the 40 chloride may be made by high temperature treatment with carbon and chloride, sulfur chloride, phosgene, carbon tetrachloride, etc. The beryllium chloride, after formation, is condensed in the cooler portions of the chlorination apparatus. After raking out from 45 the furnaces, it is stored and held ready for the electrolysis.

However, the manufacture of beryllium 50 chloride in this manner has proven a handicap to the beryllium industry, and has re-

tarded commercialization considerably. The exceedingly great tendency of beryllium chloride to hydrolyze (it is like aluminum chloride in this respect) has made impossible the conveying of the chloride from the 55 synthesizing furnaces to storage receptacles and then to the electrolysis furnaces without significant hydrolysis and therefore partial conversion of the chloride to oxide. Since much of this oxide is carried through 60 to the metal flake produced by the electrolysis, it is obvious that any procedure which could eliminate the constant danger of hydrolysis would greatly improve beryllium 65 manufacturing conditions.

A further difficulty of current beryllium manufacturing procedure is the necessity for adjusting current densities in the electrolysis cells to the beryllium chloride content. The quality of flake (size of flake is an important commercial quality factor) is largely determined by regulation of the concentration of beryllium chloride in the bath and regulation of the current densities used. Periodic addition of beryllium chloride, 70 while somewhat helpful, is an inadequate method of holding conditions constant, since the interval between each addition will of 75 itself show significant fluctuations.

I have found it possible to solve these problems and make the manufacture of beryllium a continuous process under constant, unchanging conditions, including constant beryllium chloride concentration, and with a minimum of personal attention. By completely eliminating the condensation of beryllium chloride and uniting the two steps of chloride preparation and electrolysis into one operating unit, passing the vapors resulting from the chlorination of beryllium 80 oxide directly into the bath of sodium or similar chloride (preferably with some beryllium chloride already present to lower the operating temperature), it has proven 85 possible to operate continuously without hydrolysis. The beryllium oxide or carbonate, mixed with carbon, is fed into a chlorinating furnace—I prefer a vertical silica tube externally heated, but this arrangement is 90 by no means essential to the process—and 95 100

the chlorine resulting from the electrolysis is passed through the heated mixture. This results in gaseous carbon monoxide and vaporized beryllium chloride. Passage of the mixture directly into the halide bath results in the removal of the beryllium chloride by solution in the bath, itself unchanged and in no way affecting the bath, and thence to the outside atmosphere. A further advantage 5 of the carbon monoxide passing into and over the bath is its stirring action and its acting as an inert atmosphere for the cell. Since the cell is best operated with an inert atmosphere (such as hydrogen heretofore) 10 the use of carbon monoxide for this purpose represents a definite saving.

The electrolysis proper is conducted in the standard manner, the beryllium flake, which adheres loosely to the sides of the electrolyzing pot, being periodically scraped out, freed from adhering salts as far as possible, and the remainder of the salt leached away with water. Here, however, instead of the chlorine being vented to the atmosphere, or 20 compressed for later use, as is current practice, it is trapped and passed back to the chlorination chamber, to act on fresh beryllium oxide.

It is obvious that the action of the unit is 25 almost automatic. If, for any reason, it becomes desirable to stop the electrolysis for a while, the chlorine flow will also stop and beryllium chloride manufacture will similarly automatically stop, keeping the concentration of the electrolyzing salts constant. Of course, a certain amount of loss of 30 chlorine is inevitable in practice, because of leaks, etc., but experience soon shows in the case of each unit how rapid an outside flow 35 of make-up gas is needed to keep conditions constant.

By the direct passage of the beryllium chloride in the vapor phase into the bath, all danger of hydrolysis and oxide contamination 40 is made impossible. The invention, therefore, removes this obstacle, too, from commercial beryllium manufacture.

I claim:

1. The process of preparing a bath for the 45 electrolytic isolation of beryllium comprising condensing beryllium chloride vapor by passing it into a molten bath.

2. The process of preparing a bath for the 50 electrolytic isolation of beryllium comprising condensing beryllium chloride vapor by passing it into a molten halide bath.

3. The process of preparing a bath for the 55 electrolytic isolation of beryllium comprising condensing beryllium vapor by passing it into a molten chloride bath.

4. The process of preparing a bath for the 60 electrolytic isolation of beryllium comprising condensing beryllium chloride vapor by passing it into a molten bath of sodium chloride.

5. The process of preparing a bath for the

electrolytic isolation of beryllium comprising condensing beryllium chloride vapor by passing it into a molten bath of sodium and beryllium chlorides.

6. The process of manufacturing beryllium 70 comprising forming beryllium chloride, condensing the beryllium chloride vapor by passing it into a molten bath and subjecting said bath to electrolysis.

7. The process of manufacturing beryllium 75 comprising forming beryllium chloride under essentially anhydrous conditions, condensing the beryllium chloride vapor by passing it into a molten halide bath and subjecting said bath to electrolysis.

8. The process of manufacturing beryllium 80 comprising forming beryllium chloride under essentially anhydrous conditions, condensing the beryllium chloride vapor by passing it into a molten halide bath and subjecting said bath to electrolysis, said bath being a chloride bath.

9. The process of manufacturing beryllium comprising forming beryllium chloride under essentially anhydrous conditions, condensing 90 the beryllium chloride vapor by passing it into a molten halide bath and subjecting said bath to electrolysis, the bath being one of sodium chloride.

10. The process of manufacturing beryllium comprising forming beryllium chloride under essentially anhydrous conditions, condensing the beryllium chloride vapor by passing it into a molten halide bath and subjecting 100 said bath to electrolysis, the bath being a mixture of sodium and beryllium chlorides.

11. The process of manufacturing beryllium which comprises passing beryllium chloride vapor into a halide bath and subjecting 105 said bath to electrolysis.

12. The process of manufacturing beryllium which comprises passing beryllium chloride vapor into a halide bath and subjecting said bath to electrolysis, the bath being a chloride bath.

13. The process of manufacturing beryllium which comprises passing beryllium chloride vapor into a halide bath and subjecting 110 said bath to electrolysis, the bath being one of sodium chloride.

14. The process of manufacturing beryllium which comprises passing beryllium chloride vapor into a halide bath and subjecting said bath to electrolysis, the bath being a mixture of sodium and beryllium chlorides.

15. The process of manufacturing beryllium comprising the passing of chlorine resulting from the electrolysis of a bath of beryllium chloride dissolved in a halide or mixture of halides of metals more electro-positive, overheated beryllium compounds, in the presence of a reducing agent, and passing the resulting vaporized beryllium chloride into the electrolyzing bath.

16. The process of producing beryllium

which comprises chlorinating beryllium oxide, bringing the beryllium chloride into solution in the bath and electrolyzing the bath.

6 In testimony whereof I have hereunto signed my name.

HARRY C. CLAFLIN.

38

**CERTIFICATE OF CORRECTION.**

Patent No. 1,861,656.

June 7, 1932.

HARRY C. CLAFLIN.

It is hereby certified that error appears in the printed specification of the above numbered patent requiring correction as follows: Page 1, line 39, for "the" first occurrence read and, and line 41, for "chloride" read chlorine; and that the said Letters Patent should be read with these corrections therein that the same may conform to the record of the case in the Patent Office.

Signed and sealed this 12th day of July, A. D. 1932.

M. J. Moore,  
Acting Commissioner of Patents.

(Seal)

40

45

50

55

60

which comprises chlorinating beryllium oxide, bringing the beryllium chloride into solution in the bath and electrolyzing the bath.

6 In testimony whereof I have hereunto signed my name.

HARRY C. CLAFLIN.

38

**CERTIFICATE OF CORRECTION.**

Patent No. 1,861,656.

June 7, 1932.

HARRY C. CLAFLIN.

It is hereby certified that error appears in the printed specification of the above numbered patent requiring correction as follows: Page 1, line 39, for "the" first occurrence read and, and line 41, for "chloride" read chlorine; and that the said Letters Patent should be read with these corrections therein that the same may conform to the record of the case in the Patent Office.

Signed and sealed this 12th day of July, A. D. 1932.

M. J. Moore,  
Acting Commissioner of Patents.

(Seal)

40

45

50

55

60

**CERTIFICATE OF CORRECTION.**

**Patent No. 1,861,656.**

**June 7, 1932.**

**HARRY C. CLAFLIN.**

**It is hereby certified that error appears in the printed specification of the above numbered patent requiring correction as follows: Page 1, line 39, for "the" first occurrence read and, and line 41, for "chloride" read chlorine; and that the said Letters Patent should be read with these corrections therein that the same may conform to the record of the case in the Patent Office.**

**Signed and sealed this 12th day of July, A. D. 1932.**

**(Seal)**

**M. J. Moore,  
Acting Commissioner of Patents.**